

## UNITED STATES PATENT OFFICE

2,302,939

## CLEANING ROLLED MAGNESIUM ARTICLES

Herbert K. De Long, Midland, Mich., assignor to  
The Dow Chemical Company, Midland, Mich.,  
a corporation of Michigan

No Drawing. Application January 17, 1941,  
Serial No. 374,894

10 Claims. (Cl. 148—8)

This invention relates to an improved method of removing oxide mill scale from the surfaces of rolled articles of magnesium and magnesium-base alloys.

In fabricating magnesium and magnesium-base alloys by rolling, the rolled articles frequently tend to pick up particles of mill scale, which usually appear as scattered specks or imperfections in the rolled surface. This scale, which consists chiefly of magnesium oxide and its hydrates, finely-divided magnesium metal, and carbon or carbonized oily lubricant, and will for present purposes be termed "oxide scale," adheres tenaciously to the base metal, and cannot easily be dislodged by mechanical means without marring the metal surface. Removal of the scale is important, however, since the particles serve as centers of accelerated attack if the metal is exposed to corrosive influences, and also produce blemishes when the metal is chemically treated to provide a protective surface finish.

Known chemical methods of removing the oxide mill scale generally involve pickling the rolled magnesium article in a solution of an inorganic acid, such as hydrochloric, nitric, or sulfuric acid, or mixtures thereof with chromic acid. Unfortunately, these methods, while of some value, are disadvantageous in that the acid attacks the base metal more rapidly than it does the oxide scale. As a result, the scale is not entirely removed unless the time of pickling is prolonged, with consequent great loss of metal, and in any case the scaled portions of the surface, after cleaning, appear as raised areas on the pickled article, imparting a mottled appearance thereto. Moreover, the pickling acids mentioned tend in use to become inhibited and lose their activity, so that frequent expensive replacement is necessary.

In view of these difficulties, it is an object of the present invention to provide a simple, effective and inexpensive method of removing oxide mill scale from the surfaces of rolled articles of magnesium and magnesium-base alloys.

The invention is based upon the discovery that aqueous solutions of water-soluble organic carboxylic acids, unlike those of inorganic acids, attack oxide mill scale much more rapidly than they do magnesium metal. Accordingly, by using such acids, oxide scale can be effectively removed without damage to the base metal. Moreover, the acids have a long effective life, and need be replaced only at infrequent intervals.

The carboxylic acids most suitable in the process of the invention are oxalic acid, aliphatic

carboxylic acids, such as formic, acetic, and propionic acids, and hydroxy aliphatic carboxylic acids, such as lactic, citric, and tartaric acids. Acetic, citric, and tartaric acids are particularly effective. The proportion of acid used in the aqueous cleaning solution may range from 0.2 to 50 per cent by weight or more, although concentrations of 5 to 15 per cent are most satisfactory. The cleaning process is customarily carried out at room temperature, although other temperatures up to the boiling point of the solution may be used.

In practice, the magnesium or magnesium-base alloy articles to be cleaned of oxide scale is first degreased, if necessary, and is then immersed in or otherwise subjected to the action of the carboxylic acid solution for a time sufficient to remove the scale, but insufficient to permit any substantial attack on the metal. Prolonged immersion is to be avoided. In general, at room temperature, immersion times of 0.2 to 1.0 minute are adequate, 30 seconds being especially satisfactory with acetic and citric acids. After cleaning, the metal is rinsed to remove the acid solution, and is then ready for use.

The process of the invention is especially advantageous in removing mill scale from rolled articles formed of those magnesium-base alloys which contain a small proportion of manganese as the predominating alloying element, e. g. alloys consisting of 98.5 per cent magnesium and about 1.5 per cent manganese.

It has also been found that in processes in which a protective finish is applied to the surface of rolled articles of magnesium and magnesium-base alloys by subjecting the articles to the action of an aqueous coating solution adapted to react chemically with the metal surface to form thereon a corrosion-resistant coating, a pretreatment of the article by immersing it in an aqueous solution of an organic carboxylic acid is desirable. When the pretreatment is carried out, particularly by immersion in an aqueous solution of oxalic acid, an aliphatic carboxylic acid, such as acetic acid, or a hydroxy aliphatic carboxylic acid, such as citric acid, the protective finish subsequently applied has a greater resistance to corrosion than that produced when the pretreatment is omitted. The carboxylic acid dip is especially useful as a preliminary to the production of protective finishes with acidic chromate solutions, such as a nitrate-chromate bath (Navy Aeronautical Specification M-303a).

It is to be understood that the foregoing de-

scription is illustrative rather than strictly limitative of the invention.

I claim:

1. A method of removing carbonized oil containing oxide mill scale from the surfaces of rolled articles of magnesium and magnesium-base alloys which comprises subjecting the article to the action of an aqueous solution of a water-soluble organic carboxylic acid for a time sufficient to remove the scale but insufficient to permit any substantial attack on the metal.

2. A method of removing carbonized oil containing oxide mill scale from the surfaces of rolled articles of magnesium and magnesium-base alloys which comprises immersing the article in an aqueous solution of a carboxylic acid selected from the class consisting of oxalic acid, aliphatic carboxylic acids, and hydroxy aliphatic carboxylic acids for a time sufficient to remove the scale but insufficient to permit any substantial attack on the metal.

3. A method according to claim 2 wherein the acid is acetic acid.

4. A method according to claim 2 wherein the acid is citric acid.

5. A method according to claim 2 wherein the acid is tartaric acid.

6. A method of removing carbonized oil containing oxide mill scale from the surfaces of rolled articles of magnesium-base alloys containing a small proportion of manganese as the predominant alloying element which comprises immers-

ing the article in a 5 to 15 per cent by weight aqueous solution of acetic acid at room temperature for 0.2 to 1.0 minute.

7. A method of removing carbonized oil containing oxide mill scale from the surfaces of rolled articles of magnesium-base alloys containing a small proportion of manganese as the predominant alloying element which comprises immersing the article in a 5 to 15 per cent by weight aqueous solution of citric acid at room temperature for 0.2 to 1.0 minute.

8. In a method for producing a protective finish upon the surface of rolled articles of magnesium and magnesium-base alloys having a carbonized oil-containing oxide mill scale on the surface thereof wherein the article is subjected to the action of an aqueous coating solution adapted to react chemically with the metal surface to form thereon a corrosion-resistant coating, the step which comprises immersing the article in an aqueous solution of a carboxylic acid selected from the class consisting of oxalic acid, aliphatic carboxylic acids, and hydroxy aliphatic carboxylic acids for a time sufficient to remove scale but insufficient to permit any substantial attack on the metal, prior to subjecting the article to the action of the coating solution.

9. A method according to claim 8 wherein the carboxylic acid is acetic acid.

10. A method according to claim 8 wherein the carboxylic acid is citric acid.

HERBERT K. DE LONG.